

Nov. 9, 1943.

E. R. GADD ET AL.

2,334,081

## MANUFACTURE OF NITRIDED STEEL ARTICLES

Filed Nov. 14, 1939



Fig. 2.



Inventors  
Ernest R. Gadd  
Harry Keates  
by Wilkinson & Mawhinney  
Attorneys.

## UNITED STATES PATENT OFFICE

2,334,081

## MANUFACTURE OF NITRIDED STEEL ARTICLES

Ernest Reginald Gadd and Harry Keates, Bristol, England, assignors to The Bristol Aeroplane Company Limited, Bristol, England, a British company

Application November 14, 1939, Serial No. 304,418  
In Great Britain November 12, 1938

5 Claims. (CL 148—4)

This invention relates to the manufacture of nitrided steel articles of the kind which are made of austenitic steel and case-hardened by a nitriding process. Owing to the hardness of the nitrided case the article must be finished practically to size before nitriding, and this is done by machining and grinding. These operations have the effect of work-hardening the surface material, destroying its austenitic structure and replacing it by another structure, such as 10 martensite, which is not responsive to nitriding. Further, the machining and grinding operations and exposure to the atmosphere cause an oxide film to form on the work-hardened surface, still further increasing its resistance to 15 nitriding.

In order to enable the nitriding process to be carried out it is therefore necessary to remove the resistant oxide film and work-hardened surface. According to the present invention, a method of treating the article prior to nitriding consists in immersing it in an electrolytic bath, etching it anodically to replace the resistant oxide film and work-hardened surface by a 20 passive oxide film and then etching it cathodically to remove the passive film.

It is found that the passive film produced by the anodic treatment renders the article susceptible to the nitriding process but that the presence of this film makes necessary such a 25 high temperature for the nitriding process that pitting and distortion of the articles are produced. The effect of the cathodic treatment, by removing the passive film, is to enable a lower temperature to be used for the nitriding 30 process.

A specific embodiment of the invention will now be described as applied to a process for the manufacture of sleeve-valves for controlling the ports of a sleeve-valve internal-combustion engine. In the accompanying drawing:

Figure 1 is a sectional elevation of the electrolytic bath according to the invention, and

Figure 2 is a plan view.

After the sleeve 10 has been machined and ground it is suspended as shown in Figure 1, with its axis vertical, by means of hooks 11 which engage the ports 12 in the sleeve and are fastened to a cross-bar 13 of insulating material which rests on the edges of a liquid container 14.

A rod-shaped electrode 15 of metallic lead is supported with its axis coinciding with the axis of the sleeve as shown. The rod is supported by a bracket 16 of insulating material which is fastened by bolts 17 to the lug 18 which, when

5 the sleeve is assembled in the engine, transmits the driving movement from the driving mechanism to the sleeve. The bolts 17 provide a convenient electrical connection between the conductor 19 and the sleeve, the sleeve being electrically insulated from the rod 15 by the insulating bracket 16. At the sides of the sleeve rectangular lead plates 20 are also supported in the container 14, being connected by conductors 21 to a bus-bar 22, to which the rod 15 is connected in like manner.

The container 14 is filled with an electrolyte comprising potassium bichromate in dilute sulphuric acid. The bath is prepared by adding from 42 to 56 parts by volume of commercial concentrated sulphuric acid to sufficient water to make up 100 parts by volume of dilute acid. Owing to the fact that the concentrated acid is hydroscopic and contains water, the concentration of the dilute acid will be from 30% to 40% by volume of pure acid, the lowest concentration being preferred. From 1 to 3 parts by weight of potassium bichromate is added to sufficient of the dilute acid to make up 100 parts by weight of the bath.

Anodic etching of the sleeve is effected by connecting the conductor 19 to the positive pole of a source of direct current. As shown in Figure 2 the positive and negative supply conductors 23 and 24 respectively are connected either to the bus-bar 22 and conductor 19 respectively or vice versa by adjustment of a suitable change-over switch 25. For anodic etching the switch 25 is adjusted to the position shown in full lines so that the sleeve is connected to the positive pole and the lead rod 15 and lead plates 20 are connected to the negative pole. Current is passed for from four to eight minutes, six minutes being the preferred time, the current density being between 0.75 and 0.85 ampere per square inch of sleeve. Thus, for a sleeve of 13" length and 5 1/4" internal diameter, the current used is between 350 and 400 amperes. However, the range of current density may vary from 0.5 to 1.0 ampere per square inch which, with a sleeve of the dimensions given above, means a current of from 250 to 500 amperes.

The switch 25 is then moved to the dotted line position whereby the current is reversed and the sleeve is etched cathodically at the same current density for about three minutes. Cathodic etching may be effected in some circumstances for a shorter period of time, not less than one minute. The effect of the cathodic

etching, as above explained, is that the passive oxide film is removed.

The etching process is followed by nickel plating of those parts which are not to be nitrided. In some circumstances the parts which are to be nitrided are copper-plated. The sleeve is now placed, together with other etched sleeves, in suitable containers which are moved into a furnace where they are subjected to the action of an atmosphere of ammonia at 550° C. for 72 hours. If the sleeves are not subjected to the cathodic etching above described, the temperature of the nitriding treatment has to be raised to 620° C. to produce the same case. The lower temperature has the advantages that it reduces the distortion of the sleeves, reduces the amount of pitting of the nitrided layer and lengthens the life of the containers.

The advantage of the etching process according to the invention is that it is possible in some circumstances to dispense with copper-plating of the surfaces prior to nitriding; in particular, where the process is applied to the treatment of poppet-valves and other articles other than sleeve-valves.

Instead of a bath containing potassium bichromate, a bath containing glycerol may be used, the glycerol being added in the proportion of  $\frac{1}{20}$  of an ounce avoirdupois of glycerol per gallon of dilute acid.

We claim:

1. The process of surface-hardening an austenitic steel article whereof the surface has been work-hardened by machining, which process comprises the steps of etching the article anodically in an electrolytic bath to replace the work-hardened surface by a passive oxide film, then etching the article cathodically to remove the passive film and finally subjecting the article to a nitriding treatment.

2. The process of surface-hardening an austenitic steel article whereof the surface has been work-hardened by machining, which process comprises the steps of immersing the article in an electrolytic bath, etching the article anodically

in the bath for a period of four to eight minutes at a current density of from 0.5 to 1.0 amperes per square inch of etched surface to replace the work-hardened layer by a passive oxide film, reversing the direction of the current for a period of from one to three minutes to etch the article cathodically and remove the passive oxide film, removing the article from the bath and subjecting the article to a nitriding treatment.

10 3. The process of surface-hardening an austenitic steel article whereof the surface has been work-hardened by machining, which process comprises the steps of immersing the article in an electrolytic bath comprising potassium bichromate in an aqueous solution of sulphuric acid in the proportion of from 1 to 3% by weight of potassium bichromate, etching the article anodically in the bath to replace the work-hardened surface by a passive oxide film, reversing the direction of the current to etch the article cathodically and remove the passive oxide film, removing the article from the bath and subjecting the article to a nitriding treatment.

20 4. The process according to claim 3 wherein the aqueous solution of sulphuric acid has a concentration in the order of 30 parts by volume of pure sulphuric acid to 70 parts by volume of water.

25 5. The process of surface-hardening an austenitic steel article whereof the surface has been work-hardened by machining, which process comprises the steps of immersing the article in an electrolytic bath comprising glycerol in an aqueous solution of sulphuric acid in the proportion of about  $\frac{1}{20}$  of an ounce of glycerol per gallon of the solution, etching the article anodically in the bath to replace the work-hardened surface by a passive oxide film, reversing the direction of the current to etch the article cathodically and remove the passive oxide film, removing the article from the bath and subjecting the article to a nitriding treatment.

40

45

ERNEST REGINALD GADD  
HARRY KEATES.